

Patented July 7, 1925.

1,545,385

# UNITED STATES PATENT OFFICE

EDGAR ARTHUR ASHCROFT, OF LONDON, ENGLAND.

## PROCESS FOR ELECTROLYZING FUSED METALLIC SALTS.

No Drawing. Original application filed April 10, 1922, Serial No. 551,306. Divided and this application filed February 5, 1924. Serial No. 690,875.

To all whom it may concern:

Be it known that I, EDGAR ARTHUR ASHCROFT, a subject of the King of Great Britain, residing at 32 Liverpool Street, in the city of London, England, have invented new and useful Improved Processes for Electrolyzing Fused Metallic Salts, of which the following is a specification.

My invention consists principally in an improved process for electrolyzing fused metallic salts and recovering the metals and acid radicals therefrom, and is more especially intended for use in the electrolysis of metallic chlorides such as chloride of zinc, or chloride of lead, and the recovery of the metal and chlorine.

My process can also be employed in the treatment of metal-bearing ores and other materials which when chlorinated yield metallic chloride, the said chloride (after being purified if necessary) being then subjected to electrolysis for recovery of the metal and chlorine.

My invention is hereinafter described as applied to the electrolysis of zinc chloride, but I may use it for the decomposition of any other suitable salt and also for the production of alloys from mixtures of chlorides, or other suitable salts and for the recovery of valuable constituents from metal-bearing ores and materials.

Hitherto in the electrolysis of fused salts separate couples have been employed, each couple consisting of an anode of carbon, or graphite, and a fused-metal cathode arranged within a container for the fused materials.

According to my present invention the electrolysis of the fused salt, or salts, for the separation and recovery of the metallic and other components, is effected in a multiple-couple electrolyzer comprising a series of closely-spaced electrodes all immersed in the same body of molten electrolyte. This electrolyte may be contained in a refractory, and preferably heat-insulated, container, only the first and last of the electrodes being connected with the electric supply conductors. The inner wall of the container surrounds, or embraces, the edges of the series of electrodes, thus preventing excessive leakage of current past the edges, and passages are provided for leading off separately the metallic and gaseous products of the electrolysis. The electrodes may,

if desired, be all of the same composition, for example of compressed carbon, or graphite, and any convenient number of couples may be employed, the opposed surfaces of any two adjacent electrodes and the intervening space filled with electrolyte constituting what I term a couple.

Apparatus fulfilling the requirements of the process according to my present invention is described and illustrated in the specification of my application for Letters Patent Serial No. 551,306 filed April 10, 1922. For the purpose of description I will presume that zinc chloride is treated.

The fused zinc chloride, preferably at a temperature of about 350° to 400° centigrade as this prevents "fuming" of the fused salt is introduced into the said apparatus.

During electrolysis the electrolyte is maintained at a temperature between 420° and 600° centigrade, preferably 450° to 500° centigrade. If it be desired to increase the conductivity, I may add to the zinc chloride a suitable proportion of chloride of potassium, chloride of sodium, or chloride of magnesium. The apparatus is fed with zinc chloride to replace that decomposed by the current and in this manner the said apparatus can be worked continuously for a long time. The fusion of the electrolyte may be maintained by means of the electric current, and external heat may be applied to the container, as herein-after explained. The fusion may also be maintained wholly, or in part, by applying a supplementary alternating current to the first and last electrodes of the electrolyzer, such current being more economically produced than the continuous current necessary for electrolysis.

The electrolysis sets free zinc (in the case instanced) on the upper surfaces of the electrodes and a corresponding weight of chlorine on their under surfaces. The zinc flows downwards into a reservoir and the chlorine rises to the upper part of the apparatus and the said zinc and chlorine do not come again into contact after being separated by the current. Satisfactory circulation of the electrolyte throughout the apparatus is caused by the upward flow of the gas and the downward flow of the metal.

The use of the process according to my invention results in economy of electrical energy, the use of a more convenient volt-

age, and various advantages as regards cost of construction, working and upkeep of the apparatus.

Theoretically the "chemical" voltage required for the decomposition of zinc chloride in a state of fusion is approximately 1.6 volts and the faradajic yield, per ampere hour, 1.218 grams; therefore the minimum energy required to produce one kilogram of zinc is 1315 watt-hours exclusive of that needed to keep the electrolyte in the molten condition. For technical reasons it is preferable to keep the electrolyte fused by internal electrical heating due to extra terminal voltage, or to a supplementary alternating current. It follows that efficient insulation is a prime factor in economy. It is necessary in single-couple apparatus to employ high current density, and the loss of heat through the electrodes is considerable; consequently, in the best form of single-couple apparatus, the terminal voltage per couple is believed to be approximately three times the necessary chemical voltage, and with a current efficiency of 90 per cent the energy efficiency cannot be raised much above 30 per cent. The lower the current density employed at the electrodes, with a view to securing low terminal voltage, the more accentuated are the difficulties of practical heat conservation such difficulties being due to the increased size and inconvenient form of the apparatus designed for such a purpose. It is usually found that the economical lower limit of current density is about four, to six, amperes per square inch of electrode surface, and greater current densities have often been employed.

My aforesaid multiple-couple electrolyzer enables current densities of from two amperes to one ampere, and even less, per square inch of electrode surface, to be employed, and a low terminal voltage per couple to be obtained.

In the following claims although the process according to this invention is more especially directed to the electrolysis of zinc chloride and lead chloride the expression "metallic salt" includes not only these salts, but any metallic salt to which the process is applicable and it also covers mixtures of metallic salts, and the expression "metallic chloride" also covers mixtures of metallic chlorides.

What I claim is:—

1. In the process of electrolyzing fused metallic salts, the step of decomposing the melt simultaneously at electrolytic couples in electrical series below the surface of the fused electrolyte.

2. In the process of electrolyzing fused metallic salts, the step of decomposing the melt simultaneously at electrolytic couples in electrical series below the surface of the fused electrolyte, and gathering liberated

metal in fluid condition below the zone of electrolysis.

3. In the process of electrolyzing fused metallic salts, the step of decomposing the melt simultaneously at electrolytic couples in electrical series below the surface of the fused electrolyte, and leading off liberated gas above the surface of the fused electrolyte.

4. In the process of electrolyzing fused metallic salts, the step of decomposing the melt simultaneously at electrolytic couples in electrical series below the surface of the fused electrolyte, and circulating the fused electrolyte through the action of a product of decomposition.

5. In the process of electrolyzing fused metallic salts, the step of decomposing the melt simultaneously at electrolytic couples in electrical series below the surface of the fused electrolyte, and causing the liberated products of decomposition to pass in opposed directions through the fused electrolyte and thereby effect its circulation.

6. In the process of electrolyzing fused metallic salts, the step of decomposing the melt simultaneously at electrolytic couples in electrical series below the surface of the fused electrolyte, and maintaining an equable temperature in the zone of electrolysis by causing products of decomposition to effect a circulation of the fused electrolyte.

7. In the process of electrolyzing fused metallic salts, the step of decomposing the melt simultaneously at electrolytic couples in electrical series below the surface of the fused electrolyte, and substantially confining the flow of electric current to the immersed electrode areas and the fused electrolyte therebetween in order to minimize current leakage.

8. In the process of electrolyzing fused metallic salts, the step of decomposing the melt simultaneously at electrolytic couples in electrical series below the surface of the fused electrolyte, and heating the fused melt by supplying thereto current at a voltage above the sum of the several voltages requisite to effect electrolytic decomposition at the several couples.

9. In the process of electrolyzing fused metallic salts, the step of decomposing the melt simultaneously at electrolytic couples in electrical series below the surface of the fused electrolyte, and varying the temperature of the fused melt by varying the voltage supplied thereto above the sum of the several voltages requisite to effect electrolytic decomposition at the several electrolytic couples.

10. In the process of electrolyzing fused metallic salts, effecting multiple couple electrolysis of the fused melt at a terminal voltage of less than 3.5 volts per couple.

11. In the process of electrolyzing fused

metallic salts, effecting multiple couple electrolysis of the fused melt at a current density of not more than two amperes per square inch of electrode surface in contact with the melt.

12. In the process of electrolyzing fused metallic salts, the step of decomposing the melt simultaneously at electrolytic couples in electrical series below the surface of the fused electrolyte, and minimizing heat radiation from the melt.

13. In the process of electrolyzing fused metallic salts, the step of decomposing the melt simultaneously at electrolytic couples in electrical series below the surface of the fused electrolyte, and supplying external heat to the fused melt.

14. In the process of electrolyzing fused metallic salts, the steps of feeding the fused salts in a fluid condition but below fuming temperature to an electrolytic apparatus and effecting series multiple couple electrolysis of the melt in said apparatus.

15. In the process of electrolyzing fused metallic salts, the step of decomposing the melt simultaneously at electrolytic couples in electrical series below the surface of the fused electrolyte, and maintaining the fused electrolyte at a temperature between 420° and 600° C. during electrolysis.

16. In the process of electrolyzing fused metallic salts, the step of decomposing the melt simultaneously at electrolytic couples in electrical series below the surface of the fused electrolyte, and maintaining the fused electrolyte at a temperature between 450° and 500° C. during electrolysis.

17. The method of decomposing a fused metallic salt for the recovery of metal and acid radicle therefrom, which comprises subdividing the fused melt by a group of close-

ly spaced electrodes immersed therein, and effecting the simultaneous electrolysis of the melt between adjacent electrodes by passing current in series through the several electrodes and the intervening layers of fused electrolyte.

18. The method of decomposing a fused metallic salt for the recovery of metal and acid radicle therefrom, which comprises subdividing the fused melt by a group of closely spaced electrodes immersed therein, effecting the simultaneous electrolysis of the melt between adjacent electrodes by passing current in series through the several electrodes and the intervening layers of fused electrolyte, and separately recuperating the metal and the acid radicle resulting from the decomposition.

19. The method of treating metal bearing material, which comprises chlorinating the same to obtain metallic chloride therefrom, leading said chloride in fused condition to electrolytic apparatus, and effecting series multiple couple electrolysis of the chloride therein.

20. The method of treating metal bearing material which comprises chlorinating the same to obtain metallic chloride therefrom, leading said chloride in fused condition to electrolytic apparatus, and effecting series multiple couple electrolysis of the chloride therein, and recuperating separately the metal and acid radicle resulting from electrolytic decomposition.

In testimony whereof I have signed my name to this specification in the presence of a subscribing witness.

EDGAR ARTHUR ASHCROFT

Witness:

G. F. TYSON.